

Nov. 15, 1938.

R. G. MacPHERSON

2,136,591

## METHOD FOR MANUFACTURE OF COMPOUND AGGLOMERATE CONTAINING FUEL

Filed March 9, 1936

2 Sheets-Sheet 1



*Inventor:*

*Roy G. MacPherson,*

Dr. Henry Potts, Immuno-Histology Division  
HCCS

Nov. 15, 1938.

R. G. MacPHERSON

2,136,591

METHOD FOR MANUFACTURE OF COMPOUND AGGLOMERATE CONTAINING FUEL

Filed March 9, 1936

2 Sheets-Sheet 2



*Inventor:*  
*Roy G. MacPherson,*  
*By Harry Postlethwaite, his Atty*

## UNITED STATES PATENT OFFICE

2,136,591

## METHOD FOR MANUFACTURE OF COMPOUND AGGLOMERATE CONTAINING FUEL

Roy G. MacPherson, Framingham, Mass.

Application March 9, 1936, Serial No. 67,774

4 Claims. (Cl. 44—10)

This invention relates generally to the art of fuel production, and more specifically to a novel and improved process and apparatus for making at low coking temperature an anthracitic compounded fuel, primarily for domestic use, or the making of gas. The process is useful also for making agglomerates for use in metallurgical and other fields.

The domestic users of coal require preferably a free but steady burning fuel, that is free from dust and gives off but little smoke. Without question, properly prepared anthracite coal is the nearest approach now available to an ideal fuel for that purpose, but the commercial supply of sizes larger than silt or fines is relatively limited, and expensive.

Soft coal, of which there is an unlimited supply of varying qualities, at reasonable prices, is well adapted for steam making and kindred purposes on a large scale, but not for household use, because it lacks the qualities already recited as desirable for that purpose. Of fine sizes of both kinds of coal there is an immense quantity that cannot be used satisfactorily for domestic purposes.

Many attempts have been made to make an agglomerate or compound coal, so-called, of anthracite and bituminous fines, or slack, both separately and together, and with and without other materials, compressed with a bonding material of some kind, and in the form of briquettes, or ovoids. Such coals or fuel have some merits, but the art has never been commercially very successful. Coke made from soft coal of various kinds has long been used, but such coke usually has been the by-product of processes for distilling gases of various kinds, at high temperature, and the coke has therefore been porous, quite low in volatile content, and not entirely satisfactory for domestic use, as might be expected. Coke for domestic use should be dense in structure, and free burning.

While most bituminous coals will make a dense coke, if heated slowly, it has been found practically impossible to convert any natural bituminous coal alone into a dense, low temperature coke-like fuel immediately and rapidly. But I have discovered that a properly prepared mixture of bituminous coal and other materials or elements can be quickly and satisfactorily treated by my novel method, and thereby produce a novel fuel. So far as I have been able to ascertain, all commercial soft coals are too rich in volatile content to be handled directly. They need to be diluted with less volatile solid material,

The diluting agent may be a burnable material, as anthracite fines, or coke breeze, or semi-coke made for the purpose. Or it may even be combustible material, such as lime, ores, or even common sand.

While much time and effort have been expended in the attempt to make a satisfactory product for domestic use, from soft coal, I am convinced that one or more elements besides the soft coal are needed for satisfactory production.

The best material to be used in any given case will be determined by the particular use for which the product is to be made, and the availability of the supply of these materials.

A mixture of soft coal and anthracite fines, or crushed lump anthracite, with a suitable binder, treated primarily for fuel and not for distillation of other products, makes a very satisfactory, free and long burning material for domestic use.

Many materials may be used as binders, and their character may affect materially the resulting product. Bunker oil, starch solutions, even water, have been used. A thin tar, obtained as by low temperature coking, is a satisfactory binder.

A heavy coal tar usually facilitates the blending power of a compound, and decreases the amount of bituminous coal to be used.

Molding of the mixture in some form is desirable in the making of domestic fuel, as it increases the compactness of the original mixture, and renders it more convenient for subsequent treatment. Accordingly, the present invention is directed to the production of an improved, novel compound fuel, by a novel process and apparatus.

In the drawings of one embodiment of my novel apparatus for carrying out my improved process described and illustrated herein:

Fig. 1 is a longitudinal section, with parts in elevation, of one embodiment thereof;

Fig. 2, a vertical cross section on line 2—2 of Fig. 1, looking toward the right; and

Figs. 3 and 4, modified forms, respectively, of the apparatus shown in Fig. 1.

I first mix my materials in any suitable manner, the proportions of the various ingredients depending upon the character of the various individual materials used and the type of product desired. Anthracite fines is inexpensive and readily obtainable, and yard screenings are very satisfactory for use with bituminous coal. I prefer that the dry ingredients shall be ground or classified to pass a 10 mesh screen.

When anthracite silt is used with the soft coal, the finer the anthracite silt the greater the per-

centage of soft coal that must be used within practical limits. For example, I have found that 30 parts of soft coal and 70 parts of yard screenings, as usually obtained locally, with 8 parts of light tar, all by volume, made a satisfactory combination. These proportions, however, will vary according to the degree of fineness of the materials and the kind of tar used.

After mixing the material A, Fig. 1, it is preferably fed to an endless conveyor 1, travelling on a driving roll 2 and pressure roll 3, and driven from any suitable means, not shown. I have discovered that there is a distinct advantage in treating my product in the form of a ribbon, or elongated sheet. The cost of manufacture is relatively low, and the process may be substantially continuous.

Immediately above and cooperating with the roll 3 is a second pressure roll 4, mounted adjustably to vary the amount of pressure as desired, and controlling the thickness of the ribbon of material passing through the rolls.

The conveyor 1 delivers the mixture upon a table 5, suitably secured, as by securing its flanged ends 6 to the end walls of a retort, or closed chamber 7, with a non-oxidizing atmosphere around the material, and of kettle iron, chrome iron, or other suitable material, and of proper length, say 20 to 30 feet.

30 The retort is properly housed in a brick or other setting 8, with a front wall 9, fire arch 10, baffles 11, as needed, and rear wall 12, forming a combustion chamber with a flue 12a leading to a chimney, not shown. The retort housing is provided with ports 13 for supplying fuel gas, also a nozzle 14 for gas, if desired, and again may have an oil burner 15 of convenient type and size, or the combustion chamber may be heated in any of the ways of engineering practice.

40 This retort has, at its rear end, a downwardly inclined chute 17, or discharge passage, leading to a combined storage and curing hopper 18, or other receptacle, suitably supported, with one or more outlets 19 for drawing off any gaseous products or vapor, and at the hopper's lower end, it has a discharge outlet 20, provided with any suitable valve for substantially excluding the air from the hopper 18. This valve may be a cone-shaped element 21, operated by a rod 22 extended through the hopper top, and pivoted on a post 24, and provided with a weight or other means for causing the valve to remain normally closed.

50 The hopper 18 may discharge into a second similar hopper 25, also closed by a suitable valve 26, conveniently controlled, as by a lever 27, the purpose being ordinarily not to have more than one of these valves 21 or 26 open at the same time.

It has been proposed, among other methods, to extrude a coal compound or mixture under 60 pressure through a tube subjected to substantially a coking temperature, so that the extruded compound would be coked when discharged. This plan, however, has many disadvantages and difficulties. It has been found by experience difficult 65 to cause the molded compound to flow and extrude continuously without frequent interruption, thus causing shut-downs of the machine.

70 Briquettes have been made and carbonized, but this process is expensive and difficult; it requires means to produce tremendous pressure, and it is difficult to maintain an airtight seal to the retort while feeding the briquettes to it, and it is exceedingly hard to apply a proper temperature to the briquettes, as they disintegrate with application of high heat, and again because, at coking

temperatures they will fuse together, unless well separated. Unless they can be so treated, they make an inferior fuel, as compared to my novel product, as they will disintegrate on the fire before they are consumed, and burn with a smoky flame. I have discovered that by compressing the material into a wide ribbon, or into an essentially continuous sheet of desired width, bonded to hold its shape until the exterior surface sears over sufficiently to ensure its final form, and then 10 treating it at so-called low temperature of approximately 1400 to 1600° F., it is cheaper, and far more satisfactory as a compound fuel than any that I know of.

15 The material, Fig. 1, after passing between the compressing rolls onto the plate 5, is deposited upon a suitable endless conveyor 28, as a woven wire belt on rollers 29, suitably driven as by an exterior drive belt 31, from and by driving elements not shown. The belt 28 may travel over 20 idlers 32, if desirable for support.

25 As the material is fed to the plate 5, after being compressed to a suitable thickness, say one to two inches, a hinged, or spring, cover 33 presses lightly thereon, to help keep it from buckling, if so inclined, and to practically prevent the ingress of air to the retort, and the material then passes through the retort 7, which is properly heated, say to about 1400° F. As the sheet of material approaches the forward end of the retort, a star 30 wheel 34, driven by any means, not shown, or any other convenient device, may mark and crease the sheet regularly to an extent sufficient to help cause the sheet to break into pieces of fairly uniform size, as they drop into the hopper 18, or in 35 subsequent handling.

40 By closing the valve 26, and discharging the fuel into the hopper 25 through valve 21, only a minimum amount of air will be admitted to the hopper 18 and retort 7. By closing the valve 21 and opening the valve 26, the fuel may be discharged from the hopper 25 into a car or other receptacle, without admitting more than a small quantity of air through the valve 21.

45 The cycle of operation of valves 21 and 26 may be regulated to suit the manufacturing conditions.

50 With temperature of approximately 1400° F., the mixture should yield its volatile products to the desired extent, and in effect coke satisfactorily in about 13 to 15 minutes in the retort.

55 By the foregoing process, the bituminous coal will part with some of its volatile content, and combine with the anthracite fines to form a dense mass, and I can continuously, and at low cost, produce a dense anthracite agglomerate or compounded fuel of convenient sized pieces, free and long burning, having a heating value essentially equivalent to that of the best grades of anthracite, and burning with no hard clinkers. The ash content may be regulated by the selection of suitable raw materials.

60 It is further to be understood that the actual arrangement of the elements of the apparatus used may be varied. For example, Fig. 3, the pressure rolls 3, 4, may be located within the retort, and kept cool, if desired, through the means of hollow shafts 35, carrying water or steam therethrough.

65 Another variation which may be used is shown in Fig. 4, wherein the material is compressed and formed into a sheet by means of a suitable press 36, operated by either toggles, cylinder and piston means 37, or otherwise, and resulting in an 70

intermittent, yet substantially continuous feeding motion of the ribbon of material.

Reasonable variation in the length of time required for the material to travel through the retort may be accomplished by adjustment of speed of the conveyor, or by allowing the material upon discharge into the hopper 18 to remain therein and mull in its own heat for the desired time. Small quantities of air may be admitted here, or 10 into the hopper 25, to support a partial combustion, and thus furnish additional heat for treatment, if desired.

My invention is not restricted to the particular form or embodiment of means for practising it 15 herein shown.

I claim:

1. The process of making compounded smokeless fuel comprising mixing about ten to thirty parts of comminuted coking coal with about 20 ninety to seventy parts of comminuted non-coking coal and enough volatile liquid lubricating medium to serve as a temporary binder without substantially changing its character as a dry mixture, compressing the mixture essentially cold to 25 form a self-sustaining continuous strip of approximately the density of an anthracite coal product, freely supporting the compacted strip while passing it through a heating zone containing substantially no oxygen in the surrounding 30 atmosphere at a coking temperature for a period sufficient to volatilize and coke the binder and part of the coal thereby causing the coking and non-coking coal to agglomerate in a hard dense coke-like mass having a specific gravity approximating that of the non-coking coal used, said mass containing sufficient volatile matter to be 35 free burning in domestic heaters, and separating said mass into convenient size pieces for transportation and use.

40 2. A continuous process of agglomerating coking and non-coking comminuted solid material comprising mixing a smaller proportion of coking material and a larger proportion of non-coking material with sufficient volatile liquid to serve 45 as a temporary binder when compacted, rolling the mixture without preheating to compress it into a self-sustaining continuous strip with a density of the order of the average of non-cokable constituents in the raw state, freely supporting

the strip thus formed while conveying it through a non-oxidizing heating zone at a coking temperature for a sufficient time to volatilize the binder and sinter together the coking and non-coking material in a hard dense mass, and separating said mass into fragments of desired size. 5

3. A continuous process of agglomerating coking and non-coking comminuted solid material comprising mixing a smaller proportion of coking material and a larger proportion of non-coking material with sufficient volatile liquid to serve as a temporary binder when compacted, pressing and scoring the mixture without preheating to compress the same into a self-sustaining continuous strip with a density of the order of the 10 average of non-cokable constituents in the raw state and containing depressions at regular intervals, freely supporting the strip thus formed while conveying it through a non-oxidizing heating zone at a coking temperature for a sufficient time 15 to volatilize the binder and sinter together the coking and non-coking material in a hard dense mass, and separating said mass into fragments along lines of fracture corresponding to said 20 depressions. 25

4. A process of making a dense solid agglomerate containing carbon uniformly distributed throughout the mass, comprising mixing coking coal in lesser amount and non-coking solid material in greater amount with a sufficient amount of liquid binder to hold the mixture together without changing its dry character when compacted, continuously feeding and compacting the mixture without preheating, and controlling the degree of compacting to obtain a density of product of the 30 order of the average of the non-cokable constituents in the raw state, exposing the compacted material for a substantial length of time before 35 coking it, conveying said material through an oxygen free atmosphere in a coking zone at a 40 controlled rate of speed and while free from restraint subjecting it to a temperature sufficient to cause the volatilization and coking of the binder and coking coal to form a dense solid agglomerate containing solid carbonaceous material and a 45 minimum amount of volatile material suitable for charging to a furnace. 45

ROY G. MACPHERSON.